

July 28, 1925.

1,547,787

F. H. CHAPIN

SHRINK HEAD CASING

Filed April 20, 1925

2 Sheets-Sheet 1



Fig. 2.



Fig. 1.

Fred H. Chapin,  
By Hull, Brock West,  
Attest.

July 28, 1925.

1,547,787

F. H. CHAPIN

SHRINK HEAD CASING

Filed April 20, 1925

2 Sheets-Sheet 2



Fig. 6.



Fig. 5.



Fig. 4.



Fig. 3.

Inventor

Fred H. Chapin,  
By Hull, Brock & West,  
Atty's.

## UNITED STATES PATENT OFFICE

FRED H. CHAPIN, OF CLEVELAND, OHIO, ASSIGNOR TO THE BOURNE-FULLER COMPANY, OF CLEVELAND, OHIO, A CORPORATION OF OHIO.

## SHRINK-HEAD CASING.

Application filed April 20, 1925. Serial No. 24,685.

To all whom it may concern:

Be it known that I, FRED H. CHAPIN, a citizen of the United States, residing at Cleveland, in the county of Cuyahoga and State of Ohio, have invented a certain new and useful Improvement in Shrink-Head Casings, of which the following is a full, clear, and exact description, reference being had to the accompanying drawings.

- 10 This invention relates to what are commonly known in the art of ingot casting, as feeders, sink heads, hot tops, or more properly shrink-head casings for ingot molds.
- 15 In the casting of steel ingots by the most approved methods, provision is made in the molds for maintaining in a molten condition on the top of the ingot while forming, a pool of metal which supplies to the 20 body of the ingot while being formed and solidified a sufficient amount of molten metal to fill the pipe or vertical cavity which forms or which would otherwise form during the operation. Molds of the 25 Gathmann type are so constructed that the metal solidifies more quickly in the lower portion than in the upper part thereof, so that the so called pipe is eliminated from the lower part of the ingot while being cast 30 and only a small pipe or cavity remains in the upper part of the forming ingot when the pouring operation is completed. This is true to a large extent whether the so called feeders or shrink-head casings are 35 used or not; but it is now a common practice to employ shrink head casings, inasmuch as they serve to delay the premature freezing or solidification of the top portion of the ingot by maintaining fluid, for a longer time and in a better condition, the molten metal at the top of the ingot, and thus the formation of a pipe in the body of the ingot is further prevented as the liquid steel which descends fills or prevents the formation of a pipe or a shrinkage 40 cavity which would otherwise be formed within the body of the ingot if there were a uniform rate of solidification or freezing throughout the entire molten mass. In this way the ingot is so cast that only a small pipe or cavity remains in the final product. The upper part of the ingot being cast, which contains a pool of molten metal, is sometimes called a feeder, sink head, or shrink head; and it is also common in the

art to call the heat-insulating top of the mold or that part which surrounds the pool a feeder or sink head, but this element of the mold is more properly called a shrink-head casing. It is, in fact, a part of the 50 mold, inasmuch as the upper part of the ingot is cast therein, but it is usually separable from the mold proper and made of different material.

Ordinarily heretofore shrink-head casings have been made of refractory material, such as fire clay or fire brick-material which is extremely hard and brittle, having been baked at a very high temperature and having a texture which is quite close. In order to make such casings, special plants have been required; it has not been the practice to make such casings at steel plants. Thus transportation of the casings has been necessary and the expense is correspondingly 65 increased. When in use, the fire-clay or fire-brick casings have been supported on the molds by some means which allow them to descend into the mold cavity as the ingot shrinks and solidifies. This has been found 70 necessary, as the casing adheres to the top of the ingot and, unless it is allowed to lower with the shrinking ingot, it will be broken and prematurely destroyed. When the casting operation is finished, the casing 75 remains on top of the ingot and is usually broken up by hammers or other suitable tools and thus removed from the ingot before the latter is reheated and passed to the rolls for reducing the ingot to the 80 desired shape. Quite often lumps and finer particles of clay remain on the ingot and become embedded therein while passing through the rolls, thus making flaws in the 85 rolled product which are sometimes serious. 90

Shrink-head casings made of fire-clay have rather low heat-insulating qualities, necessitating the loss of a considerable quantity of metal from the top of the ingot where the pipe or cavity occurs, it being 100 necessary to remove or crop this portion of the ingot after it and the sound portion thereof are rolled into blooms, billets, or other shapes.

It is the object of my invention to overcome the defects ordinarily found in shrink-head casings as heretofore made, and I have devised a way of making such casings of material which is not only much cheaper than fire clay or similar refractory material, 110

but which will produce casings of greater efficiency because possessing characteristics which entirely eliminate some of the difficulties heretofore encountered in the use of 5 clay casings.

I have found that if blast furnace slag is properly prepared and mixed in ordinary water in proper proportions with commercial Portland cement, it may be molded into 10 proper shape for use as shrink-head casings and that, if the surface of such a casing be treated with a suitable substance, it will be rendered water-proof or non-absorbent of liquids or gases. This treatment of the casings 15 also prevents the formation and liberation of such gases in the interior of the casing as would produce an endo-thermic action in connection with the molten metal contacting with the casing which would result in what is known in the art as a "boil", or such a disturbance in the forming ingot as to impede or mar the proper casting of the ingot, and the formation of gases in the casing which would crack or break it. 20 My improvements are illustrated in the accompanying drawings in which Fig. 1 is a perspective view showing the upper portion of an ingot mold and a shrink-head casing made in accordance with my invention; Fig. 2 a vertical sectional view of an ingot mold with a shrink-head casing supported in operative relation thereto and thereon, the section being taken on the line 2--2 of Fig. 6; Fig. 3 a detail in vertical section of 25 a portion of the shrink-head casing showing how its walls are treated in the manner hereinafter specified; Fig. 4 a central vertical sectional view through the mold and casing, showing how the molten metal rises 30 into the casing during the pouring operation; Fig. 5 a view similar to Fig. 4 showing how the ingot, during shrinkage, draws away from the casing without bodily moving the latter; and Fig. 6 is a top plan view 35 of the ingot mold, with the said shrink-head casing resting thereon.

The particular shape of the casing is not essential. Various shapes may be used, but that illustrated in the drawing is preferred. 40 As shown, the casing B is generally rectangular in horizontal cross section. The lower part of the casing is rounded at the four corners thus producing a lower part c which is adapted to enter the mold cavity and 45 shoulders d which are adapted to rest on the top of the mold and thus support the casing. While I prefer to mold the casing in one integral piece, it may be made in sections. When the mold is of large size, a 50 sectional casing may be found preferable. The ingot mold A shown herein is of the Gathmann type, and the ingot therein is indicated at I.

While heretofore shrink-head casings have 55 ordinarily been made of refractory material,

such as fire clay baked at a high temperature in a special plant generally remote from the steel plant, the casings made in accordance with my invention are made of relatively low-refractory material, baked or 70 hardened at a relatively low temperature, and may be made at the steel plant, inasmuch as I employ furnace slag as a principal ingredient of the casing and combine such slag with a suitable proportion of commercial Portland cement, which is readily obtainable. Blast furnace slag gives the best results, although open hearth or other 75 slag may be used.

In my application for patent filed April 20, 1925, No. 24,684, I have described and claimed the method of preparing, forming and treating the material to produce shrink-head casings having the desired characteristics. Briefly stated, the method consists in 80 grinding or crushing ordinary slag taken from the dump, screening this product through  $\frac{1}{4}$  inch mesh to eliminate the large lumps, then mixing the screened slag with commercial cement, preferably in the proportions of about 7 parts by weight of slag to about 1 part by weight of cement, although these proportions may be somewhat varied. By this treatment, the cement and 85 slag are thoroughly mixed and blended while dry, and then a suitable amount of ordinary cold water is added to produce a stiff moist product which is then placed in suitable molds and rammed or tamped in the usual way until the desired shape is 90 obtained. The casings are then preheated, or heated at a relatively low temperature in a suitable furnace to about 200° to 250° F. for about 12 hours. In this way all free 95 moisture is eliminated and the setting of the cement is hastened. The cement as it sets acts as a binder, and I preferably use commercial Portland cement for such binder, although other materials might be used for 100 this purpose with fairly good results. When 105 dried and baked at the temperatures specified, the casing is rendered porous and in 110 good condition to receive the impregnating liquid or substance which serves to prevent 115 the formation and liberation of deleterious gases from the casing when the latter is subjected to the intense heat of the ingot while 120 being formed. For this purpose I preferably employ a substance sold as "goulac," well known to foundry men and which consists mainly of organic matter (cellulose), with 125 the following additional ingredients:

Aluminum oxide ( $Al_2O_3$ ), ferric oxide ( $Fe_2O_3$ ), manganese oxide ( $Mn_2O_3$ ), calcium oxide ( $CaO$ ), magnesium oxide ( $MgO$ ), sulphur (s).

The cellulose in the "goulac" is that obtained from the dried liquor from the manufacture of sulphite pulp. A non-organic compound, such as magnesium fluosilicate, 130

may also be used instead of "goulac". The impregnating substance may be applied by spraying, brushing or by dipping the casing into a bath of the liquid, whereby all the walls are impregnated to a suitable distance with the impregnating substance. While good results have been obtained where the impregnation extends from  $\frac{1}{8}$  to  $\frac{3}{4}$  inch into the casing walls, it is preferable to impregnate the casing completely, as indicated by the stippling at  $\alpha$  in Figs. 1 and 3. The impregnating material serves not only to prevent the formation and liberation of gases but it also renders the casing as a whole substantially water-proof, so that it will not absorb moisture and thus render the porous casing liable to rupture or spawling through the formation of steam or gases therewithin.

After being thus treated, the casings are baked in a suitable furnace for about 12 hours, the latter being heated to a temperature of from  $600^{\circ}$  to  $800^{\circ}$  F. which, it will be observed, is not only a much lower temperature than that employed for burning fire clay but one which will not fuse the slag ingredient of the casings. When thus baked, the casings are complete and ready for use on the molds.

While I prefer to apply the impregnating substance to the entire exterior of each casing, it may be applied only to the inner walls thereof which come in contact with the molten metal of the forming ingot, and I may apply other forms of water-proofing material to other parts of the casing.

Inasmuch as the interior of each casing is porous and substantially moisture-free, it serves as a heat insulator, and the metal of the forming ingot at the top of the mold is maintained in liquid condition until the formation of the ingot is completed.

While my casing is in use, the hot molten metal which rises in it when the mold is being poured softens the inner walls of the casing, due to the fusion of the slag constituent thereof, and renders them non-adherent to the ingot, so that as the forming ingot shrinks it will draw away from the casing without imparting harmful strains thereto, the inner surface of the casing flowing with the shrinking ingot. This feature of the invention is illustrated in Figs. 4 and 5 of the drawings.

The casing, when in use, is supported at all times on the shoulders  $\delta$  and no provision is made for lowering the casing into the mold cavity to accommodate the shrinkage of the solidifying ingot, indicated at  $\alpha$ .

By reference to Fig. 4 it will be seen that the ingot has an upper portion  $i$  within the casing. At the stage illustrated in Fig. 4, the lower edge of the casing comes in contact with a ledge  $\gamma$  of the ingot, but as the ingot solidifies and shrinks it lowers or pulls

away from the casing, leaving a vacant space, indicated at  $\alpha$ . This is made possible by reason of the fact that the heat of the ingot within the casing softens the inner walls of the casing to such an extent that they become somewhat slippery, so to speak, and the upper or top portion of the ingot within the casing readily slides downwardly without moving the casing or putting any harmful strain thereon. This is quite an important feature of the invention. Furthermore, the impregnating substance prevents the swelling or spawling of the slag constituent of the casing and thus enables the ingot to free itself during its solidification and shrinkage.

My invention, while especially designed for use in connection with molds for forming steel ingots, may be employed in connection with molds of other kinds and with molds for forming other kinds of castings.

It has been stated that the plant for making the casings is conveniently located at the steel plant where the slag is found, but it is of course feasible to make the casings in plants remote from the steel plants, although this involves transportation and additional expense. In any event, by using a waste product such as slag in connection with a relatively small percentage of cement or binding material, my casings may be made very much more cheaply than can those made of fire clay; and casings made in accordance with my invention possess the beneficial characteristics, set forth hereinbefore, which are not found in casings heretofore employed.

While the slags mentioned hereinbefore will produce casings having the advantages referred to, the best results are obtained by using a slag containing a substantial proportion of magnesia.

In my application for Patent No. 758,594, filed December 29, 1924, I have claimed broadly among other things a shrink-head casing made from a mixture of furnace slag and a binder. I have also claimed broadly a shrink-head casing of refractory material treated or combined with a material capable of preventing the deleterious action of the gas producing constituents of the casing.

Having thus described my invention, what I claim is:—

1. A shrink head casing for ingot molds comprising a mixture of furnace slag and a binder and having its inner walls impregnated with a substance which prevents the deleterious action of the gas producing constituents of the mixture.

2. A shrink head casing for ingot molds comprising a mixture of furnace slag and cement and the inner walls of which contain a substance which renders inactive the gas forming constituents of the mixture.

3. A shrink head casing for ingot molds

- comprising a mixture of blast furnace slag and a binder combined with a substance which prevents the deleterious action of the gas forming constituents of the mixture.
4. A shrink head casing for ingot molds comprising a mixture of furnace slag and cement and which has its inner walls impregnated with a substance which prevents the deleterious action of the gas producing constituents of the mixture, said casing being rendered impervious to moisture throughout its entire exterior.
5. A shrink head casing for ingot molds comprising a mixture of refractory material and a binder, having its inner walls impregnated with a substance which prevents the deleterious action of the gas producing constituents of the mixture and said casing being also coated throughout its exterior to render it waterproof.
6. A shrink head casing for ingot molds comprising a mixture of blast furnace slag and Portland cement, having its inner walls impregnated with a substance which prevents the formation and liberation of gases when the casing is subjected to the intense heat of a forming ingot.
7. A shrink head casing for ingot molds made of thoroughly blended refractory material and a binder having a porous moisture free interior and water proofed outer walls.
8. A shrink head casing for ingot molds comprising a mixture of blast furnace slag and cement and having a porous interior and a water proofed outer surface.
9. A shrink head casing for ingot molds made of blast furnace slag and cement, having an inner wall, the surface of which is fusible and thus non-adherent to the forming ingot to allow the ingot to descend while shrinking without moving the casing.
10. A shrink head casing for ingot molds composed of refractory material and a binder, having inner walls which are fusible to an extent to render them non-adherent to the ingot to thus allow the hot upper end of the forming ingot to slip downward in the casing while the ingot is solidifying and shrinking.
11. A shrink head casing for ingot molds made of a mixture of refractory material and a binder having its inner walls fusible at a temperature below that of the forming ingot to thus become non-adherent to the ingot and to thus allow the upper end of the ingot to shrink in the mold without moving the casing.
12. A shrink head casing for ingot molds made of refractory material and a binder having an inner wall, the surface of which is fusible and thus non-adherent to the forming ingot to thus allow the ingot to descend in the mold while shrinking without moving the casing, said inner wall being impregnated with a substance which renders inactive the gas producing constituents of the casing.
13. A shrink head casing for ingot molds made of refractory material and a binder having a porous, moisture free interior and having its inner wall impregnated with a substance which renders inactive the gas producing constituents of the mixture, the surface of said inner walls being fusible at the temperature of the forming ingot to allow the forming ingot to slip past the casing while shrinking.
14. A shrink head casing for ingot molds made of a mixture of blast furnace slag and cement, impregnated throughout with a substance which renders inactive the gas producing constituents of the mixture, the surface of the inner walls of the casing being fusible at the temperature of the forming ingot to allow the forming ingot to slip past the casing without moving it while the ingot is shrinking.
15. A shrink-head casing for ingot molds comprising a mixture of furnace slag and cement in about the proportions of seven parts of slag to one part of cement and having its inner wall treated with a substance which prevents the deleterious action of the gas-producing constituents of said casing.
16. A shrink-head casing for ingot molds comprising a mixture of furnace slag and a binder in the proportions of about seven parts of such slag to one part of the binder and having its inner wall treated with a substance which prevents the deleterious action of the gas-producing constituents of the casing.
17. A shrink-head casing for ingot molds comprising a mixture of furnace slag and cement in the proportions of about seven parts of such slag to one part of cement, the said casing having a water-proofed exterior.
18. A shrink-head casing for ingot molds made of a mixture of refractory material and a binder and having an inner wall which is fusible at the temperature of the molten metal of the ingot and having its exterior water-proofed.

In testimony whereof, I hereunto affix my signature.

FRED H. CHAPIN.